

## UNITED STATES PATENT OFFICE

1,996,017

PROCESS FOR PRODUCING ARTIFICIAL  
SILK IN THE FORM OF SPUN CAKES

Franz Hoelkeskamp, Wuppertal-Wichlinghausen,  
Germany, assignor to American Bemberg Corporation,  
New York, N. Y., a corporation of  
Delaware

No Drawing. Application December 17, 1930,  
Serial No. 502,988. In Germany December 20,  
1929

8 Claims. (Cl. 18—54)

In the spinning of artificial silk hitherto spinning pots were used which usually had an internal diameter of 15—20 cm. and rotated at about 6,000 revolutions. These spinning pots were found to be thoroughly reliable in the production of artificial silk of the usual titre if attention was paid to their careful mounting which ensured smooth running and satisfactory spinning at the requisite high rotational speed.

However, if finer titres are spun, for example according to the cuprammonium stretch-spinning process, it is found that the winding up into spun cakes cannot any longer be effected free from trouble in the case of yarn of 60 deniers and less. The filaments are drawn into the spinning pot badly or not at all. These disadvantages would be avoided by raising the speed of revolution, but bearing in mind security in mounting, this is not possible. However, even in the case of the usual titres, a diminution in the rotational speed is of advantage from the point of view of simpler mounting.

The subject of this invention is a process for collecting artificial silk in the usual spinning pots. The process consists in weighting the fine filaments in a suitable manner before introduction into the spinning pot. Even in the case of extreme fineness, such weighted filaments are drawn smoothly into the spinning pot and are wound to a perfectly satisfactory cake.

The weighting is best effected by producing a precipitate on the fibre, the freshly-spun filament being treated with solutions of substances which react with the substances derived from the precipitating bath to form an insoluble compound. Those compounds which can interact to form comparatively heavy compounds are particularly suitable. Thus, in the case of filaments of cuprammonium silk, salts of heavy metals which, under the influence of the ammonia and copper still contained in the filament, react to form insoluble basic salts or to form hydroxides are particularly suitable. In the case of viscose filaments, which leave the spinning bath charged with sulphuric acid or sulphate solutions, an after-treatment with soluble lead salts is particularly advantageous.

The present process also enables satisfactory spun cakes to be made in spinning pots of much diminished rotational speed when spinning artificial silk filaments of the usual titre. The speed of rotation is smaller so that the spinning pot is considerably protected. Also the power required is strongly diminished and the mounting is fa-

cilitated, since the accuracy of the mounting need not be so high in the case of lower rotational speeds, for the forces acting on the bearings producing uneven running increase considerably with rising rotational speed.

After spinning, the precipitates are dissolved during the after-treatment by suitable agents, such as acids, and removed from the filaments by washing. In the processes heretofore known after-treatment with acid or the like was also necessary, so that the process according to this invention is no more bothersome.

The process will now be described in greater detail by reference to some examples.

The individual filaments of cuprammonium oxide issuing from the nozzle into a spinning vessel with flowing water as precipitating liquor are precipitated and leave the spinning vessel with a considerable copper hydroxide content. Metal salt solutions are then supplied dropwise to the filament, while being conducted over rollers, before it enters the centrifuge. The metal salt, e. g. 6 g. of commercial  $\text{CuSO}_4$  to 1 litre of water, or 7 g. of commercial  $\text{MgSO}_4$  to 1 litre of water, interacts with the substances still remaining behind from the precipitation the products whereof are insoluble salts which precipitate on the filament and are only dissolved out again in the spinning pot, into the top of which acid is introduced.

For forming the precipitate those quantities of salt solutions are preferably used which are necessary for interacting with every trace of the substances present in the filament. The metal salt solutions used react with the copper hydroxide present in the filament according to the following equations:



The process, however, is limited neither to the cuprammonium oxide process nor to the salt solutions mentioned by way of example; on the contrary, other processes and other salt solutions may also be employed. It is only necessary to choose those solutions which react with the substances on the filament and precipitate insoluble substances on the latter, thereby weighting the filament, which insoluble substances are removed only subsequently, after they have performed their task.

What I claim is:

1. In the production of artificial silk the steps of forming a thread of at most 60 deniers weighting said thread by water insoluble metallic compounds, collecting said thread in the form of a cake by a rotating spinning centrifuge and removing said insoluble metallic compounds by suitable means.
2. In the manufacture of cuprammonium silk the steps of forming a thread of at most 60 deniers, producing a precipitate of water insoluble metallic salts on said thread, collecting the thread in the form of a cake by a rotating spinning centrifuge, and dissolving the insoluble salts from the thread by suitable acid solutions.
3. In the preparation of artificial silk of fine denier, the step of weighting preformed filaments with a water-insoluble, acid-soluble heavy material, collecting the weighted filaments in a centrifuge and applying acid to the cake formed in the centrifuge.
4. In the preparation of artificial silk of fine denier by the cuprammonium process, the steps of treating the spun filaments with a material which will react with the precipitating solution to precipitate a heavy water insoluble compound upon the filaments, collecting the filaments in a centrifuge and thereafter treating them in a solution which will dissolve the insoluble compound.
5. In the preparation of artificial silk of fine

denier by the cuprammonium process, the steps of treating the spun filaments immediately after leaving the spinning bath with a solution of a salt of one of the metals of the group consisting of copper and magnesium to precipitate an insoluble salt of the metal upon the filament, collecting the filaments by centrifugal force and washing them with an acid solution.

6. In the preparation of artificial filaments of fine denier, the steps comprising precipitating a water insoluble metallic salt upon the formed filaments, collecting the filaments in a spinning cake by centrifugal force and thereafter removing the water insoluble compound.

7. In the preparation of artificial filaments of fine denier, the steps comprising extruding the filaments into a precipitating bath, treating the formed filaments with a compound which reacts with the portion of the precipitating bath retained by the filaments to deposit a water insoluble metallic compound thereon and thereafter collecting the filaments by centrifugal force and removing the insoluble compound.

8. In the production of artificial filaments of fine denier, the steps comprising weighting said filaments with a water insoluble compound, collecting the filaments in the form of a cake by a rotating centrifuge and removing said insoluble compound by suitable means.

FRANZ HOELKESKAMP.

30